

## UNITED STATES PATENT OFFICE

2,076,579

## FREE CUTTING ALLOY

Louis W. Kempf and Walter A. Dean, Cleveland,  
Ohio, assignors to Aluminum Company of  
America, Pittsburgh, Pa., a corporation of  
Pennsylvania

No Drawing. Original application December 28,  
1935, Serial No. 56,552. Divided and this ap-  
plication July 27, 1936, Serial No. 92,925

3 Claims. (Cl. 75—147)

The invention relates to aluminum base al-  
loys and is particularly concerned with aluminum  
base alloys containing magnesium and silicon.

This application is a division of our co-pending  
5 application, Serial No. 56,552, filed December 28,  
1935. Alloys disclosed but not claimed herein are  
claimed in the aforesaid co-pending application,  
Serial No. 56,552.

Aluminum base alloys containing from about  
10 0.1 per cent to 1.0 per cent of magnesium, and  
from about 0.5 per cent to about 2.5 per cent of  
silicon have heretofore been used. They are usually  
in the wrought condition since they are  
readily susceptible to mechanical deformation  
15 such as rolling, forging, or extrusion. It is possible,  
by appropriate thermal treatment, to very  
substantially improve their physical properties.  
After a high temperature solution treatment they  
do not age-harden to any great extent at room  
20 temperature but may be artificially aged by tem-  
peratures somewhat in excess of room tempera-  
ture as is well known in the art. For this reason  
these alloys may be wrought to substantially final  
form, then subjected to a high temperature solu-  
25 tion treatment, and while in a relatively soft  
condition they may be given certain final working  
steps at low temperature. Since they do not  
materially age at room temperature these finish-  
ing steps may be performed at any convenient  
30 time. They may ultimately be artificially aged if  
the maximum tensile strength, yield strength, and  
hardness are desired.

Since all commercial aluminum base alloys  
35 contain some silicon as an impurity, usually less  
than, or not greatly in excess of 0.5 per cent, it  
is to be understood that the amount of silicon  
discussed herein, and hereinafter claimed, repre-  
sents the total quantity of silicon present, and  
40 that the silicon content of the aluminum used  
should be known in order to provide a basis for  
determining the eventual composition of the  
aluminum-magnesium-silicon alloy.

There are, however, some applications wherein  
45 aluminum-magnesium-silicon alloys as herein-  
above disclosed might be conveniently and profit-  
ably used except for an inherent disadvantage  
which militates against their use in the produc-  
tion of certain articles requiring exacting ma-  
chining operations. Mechanical cutting opera-  
50 tions such as drilling, shaping, or lathe-cutting  
are successfully carried out only by using certain  
precautions which increase the cost of produc-  
tion and perhaps favor the choice of another  
metal or alloy which can be machined more  
55 readily but which is not so desirable in other

respects, as for example, in physical properties.  
When alloys are difficult to machine this disad-  
vantage becomes evident, in many cases through  
rapid wear of the cutting tool edge, so that fre-  
quent tool re-sharpening is required. Despite 5  
continual lubrication the machined surface is  
rough and irregular, and the chip has a tendency  
to form a continuous curl or spiral which often  
fouls the tool or the moving parts of the machine.  
It is immediately apparent that there is need for 10  
an alloy of good working characteristics and sat-  
isfactory physical properties, yet possessing such  
favorable machining properties that the complete  
machining operations may be performed econo-  
mically and successfully, and may be productive of 15  
a pleasing surface appearance.

Accordingly an object of our invention is the  
provision of an aluminum base alloy containing  
from about 0.1 to about 1.5 per cent of magnesium  
and from about 0.5 to 2.5 per cent of silicon, 20  
which may be readily and economically ma-  
chined.

Our invention resides in the discovery that the  
foregoing object is effected by adding at least one  
25 of the elements lead and tin to the aluminum-  
magnesium-silicon alloy. When these elements  
are added, in the proportions specified below, the  
alloys are known as free cutting or free ma-  
chining alloys because they can be machined  
30 more rapidly than similar alloys without the lead  
or tin, and yet have as good or a better finished  
surface. After an extended series of investiga-  
tions we have discovered that the elements lead  
35 and tin belong to a class of alloying elements  
which has a favorable effect upon the machining  
properties of aluminum-magnesium-silicon al-  
loys. In recognition of this effect we term lead  
and tin "free machining" elements. We have fur-  
ther discovered that the simultaneous presence of  
40 both of these elements is productive of an im-  
provement in free machining characteristics which  
is considerably greater than that caused by the  
presence of the same total amount of either one  
alone. For example, the addition of 0.5 per cent  
45 of lead and 0.5 per cent of tin to an aluminum  
base alloy containing about 0.6 per cent of mag-  
nesium and 1.0 per cent of silicon effects a greater  
improvement in machining quality than does  
the addition of 1.0 per cent of either lead or tin  
50 singly.

Since these two elements have such a favorable  
effect on the machining characteristics of alumi-  
num-magnesium-silicon alloys, it is fortunate  
that they are also of relatively low melting point,  
a fact which makes possible their addition to 55

molten aluminum in the pure state, without the intervention of so-called "rich alloys". It is also a fact that the elements lead and tin form with aluminum a series of alloys of limited liquid solubility. Within the range disclosed and claimed, however, these free machining elements may be added without unusual difficulty. We suspect that this characteristic feature of the elements lead and tin may be one of the significant factors which contribute to their free machining effect. We believe that this effect is further strengthened by distributing the free machining constituent relatively homogeneously throughout the solid matrix, since lead and tin are also practically insoluble in the solid aluminum-magnesium-silicon base alloy.

The lead or tin, if used alone, may be added in amounts between about 0.05 per cent and 6.0 per cent. If used together the total amount of free machining constituent should not be less than 0.05 per cent, and need not exceed 6.0 per cent. We have determined that the maximum limit of 6.0 per cent of free machining metal is sufficient for satisfactory commercial results, since although the free machining effect persists beyond this amount, certain of the other physical properties may be unfavorably affected.

Aluminum-magnesium-silicon alloys containing one or both of the free machining elements lead or tin may be machined more rapidly, with less tool wear, less tool sharpening, better quality of chip and better machined surface than the same base alloys without the free machining additions and as previously indicated the simultaneous presence of tin and lead is considerably more helpful to the machining quality of the alloy than an equivalent total amount of either lead or tin alone.

As a preferred alloy within the range of the respective elements disclosed hereinabove we suggest an alloy containing about 0.6 per cent of magnesium, 1.0 per cent of silicon and a total of 3 per cent of lead and tin, the balance being aluminum. For some applications which do not require a high degree of free machining quality a lesser amount of the free machining metal may be added to the alloy base, for instance 0.5 per cent of lead or 0.5 per cent of tin, or 0.75 per cent total of lead and tin.

For certain purposes, notably the improvement of tensile strength, hardness and grain structure, the alloys as hereinabove disclosed may be improved by the addition of one or more of the group of elements composed of molybdenum, vanadium, titanium, tungsten, zirconium and chromium. From 0.05 to 1 per cent of any one of these ele-

ments may be used alone, but if more than one is employed the total amount should not exceed about 2 per cent.

The free machining alloys which have been described hereinabove may be subjected to the thermal treatments well known in the art to improve their strength and hardness. We have found that a solution heat treatment and subsequent aging does not impair the free machining quality of the alloys and in many instances the treatment even tends to improve this property. For many purposes a relatively high strength and hardness are necessary to the successful performance of the machined article and hence the alloy must be heat treated. This treatment is generally applied prior to the machining operation.

As hereinabove indicated the free machining elements, by reason of their low melting point, may be added to the molten aluminum in pure metallic form. However, since some difficulty may be encountered in introducing them in the higher percentages of our disclosed range we prefer to use the method which is more fully described in U. S. Patent No. 1,959,029, issued March 15, 1934. Briefly it involves heating the melt to a somewhat higher temperature than is customary, and vigorously stirring it in excess of a critical period of time.

The term "aluminum" as used herein and in the appended claims embraces the usual impurities found in aluminum ingot of commercial grade or picked up in the course of the ordinary handling operations incident to melting practice.

We claim:

1. A free cutting alloy containing from 0.1 to 1.5 per cent magnesium, from 0.5 to 2.5 per cent silicon, from 0.05 to 6.0 per cent lead and from 0.05 to 6 per cent tin, the total amount of lead and tin being not in excess of about 6.0 per cent, the balance being substantially aluminum.

2. A free cutting alloy containing from 0.1 to 1.5 per cent magnesium, from 0.5 to 2.5 per cent silicon, from 0.05 to 6.0 per cent lead and from 0.05 to 6.0 per cent tin, the total amount of lead and tin being not in excess of about 6.0 per cent, and from 0.05 to 2 per cent of hardening metal from the group composed of molybdenum, vanadium, titanium, tungsten, zirconium, and chromium, the balance being substantially aluminum.

3. A free cutting alloy containing about 0.6 per cent magnesium, 1.0 per cent silicon, 0.5 per cent lead and 0.5 per cent tin, the balance being aluminum.

LOUIS W. KEMPF.  
WALTER A. DEAN.